

# UNITED STATES PATENT OFFICE.

ALFRED E. JURY, OF NEWARK, NEW JERSEY, ASSIGNOR, BY MESNE ASSIGNMENTS,  
TO MORGAN & WRIGHT, OF DETROIT, MICHIGAN, A CORPORATION OF MICHIGAN.

## PROCESS FOR TREATING FIBROUS MATERIAL AND THE PRODUCTS OBTAINED THEREBY.

1,356,920.

Specification of Letters Patent. Patented Oct. 26, 1920.

No Drawing.

Application filed June 25, 1919. Serial No. 306,531.

To all whom it may concern:

Be it known that I, ALFRED E. JURY, a citizen of the United States, residing at Newark, county of Essex, State of New Jersey, have invented certain new and useful Improvements in Processes for Treating Fibrous Material and the Products Obtained Thereby, of which the following is a full, clear, and exact description.

10 This invention relates to processes for treating fibrous material and to the products obtained thereby. It is more particularly directed to a process for providing fibrous materials for use for example in rubber tires or in other articles where there is excessive wear due to flexing and abrasion; and to the products obtained by such process.

One of the objects of the invention is to 20 provide a simple process of the kind described adapted to treat the fibrous material thoroughly and uniformly. Another object is to provide an efficient process of the kind mentioned adapted to prepare the 25 fibers without impairing the flexibility of materials made therefrom and practically without preventing the penetrability of such materials by rubber or similar plastic. Another object of the invention is to provide 30 an article having heightened resistance to wear which shall exhibit a marked resistance to the action of the various agents encountered in vulcanizing processes.

The invention covers both the product 35 and a method of producing same, the latter, briefly stated, comprising applying to fibrous material a lubricant in a volatile solvent, impregnating the materials, evaporating the solvent and applying a coating of rubber or 40 similar plastic substance to the so-treated fibrous material.

In carrying out the process in its preferred form, the fibrous material preferably in the form of single ply yarn is immersed 45 for approximately ten seconds in an impregnating medium serving to coat the individual fibers preferably containing the follow-

ing ingredients in about the proportions stated:

|                     |                   |     |
|---------------------|-------------------|-----|
| Castor oil          | 2 parts by weight | 50  |
| Beeswax             | 1 "               | " " |
| Carbon tetrachlorid | 97 "              | " " |

The immersion of the yarn is accomplished by passing the several strands thereof on the way to the twisting frame through a trough or pan which contains the coating medium. The pan is arranged between the spools of yarn and the rollers between which the single strands pass immediately before they are twisted together. After immersion, the yarn is subjected to pressure by rolls to remove any excess of the coating medium. The solvent is then preferably evaporated by any well-known drying method with or without the use of artificial heating means. The yarns so treated may then be twisted in the usual manner and woven into fabric or manufactured into any desired form. Rubber or other plastic material may be applied to the fibrous material in the form of fabric or otherwise. The plastic material may be applied in any well known manner, for example, by frictioning the fabric. The oil is substantially non-drying and this together with the wax serve as a lubricant and the quantity of the lubricant employed is such that the fibers are thinly coated while the spaces normally present between the individual fibers are maintained substantially open. Where the fibers cross one another the lubricant serves to prevent friction.

Although the coating solution is preferably applied to single ply yarn as mentioned above, it may also be applied to the fibrous material in other forms, for example, it may be applied after the fibrous material has been woven into fabric or twisted into cord, or while it is in the form of plied yard, or in any of the forms through which it passes at the various stages of its manufacture such as sliver or roving, or in its natural state.

It will also be observed that, although castor oil and beeswax are preferably employed together in the coating medium, good results have been obtained by the use of these substances separately, and that these substances are simply representatives of a large class of materials with which I have made experiments and which have been found suitable for the purpose mentioned, examples of these being cotton seed oil, olive oil, paraffin and carnauba. Carbon tetrachlorid is preferred as a solvent, but it has also been found that benzol, kerosene, and gasolene may be similarly used with good results.

As mentioned above, the coating of the fibers in the manner indicated appears to form lubricated joints where the fibers cross or overlie one another, and such joints reduce the internal friction and wear due to flexing and abrasion. The formation of such lubricated joints, may be brought about in a somewhat similar manner to that recited in the process above by treating fibrous material, ordinarily provided with a natural protective coating, for example, cotton with its coating of waxy material with a volatile solvent. In carrying out such process in its preferred form, the fibrous material is immersed in carbon tetrachlorid at a high temperature for a short period. The solvent is then driven off by any desired drying means. By this treatment the natural waxy material appears to be brought to a fluid or pasty condition and in this condition lubricated bonds are formed between the adjacent fibers. In carrying out this process the fibrous material may be treated in the form of threads, cords or fabric, and various solvents other than carbon tetrachlorid, such as benzol and kerosene may be employed with good results.

Coating with oil and wax in a volatile solvent effects a thorough, rapid and uniform penetration of the fiber. The uniformity of the coating is insured through the use of these materials in solution. The thoroughness of the penetration is insured by employing a volatile organic solvent. Experiment has shown that such solvent is better adapted for penetration of fibrous material than a vehicle such as water. Further with the use of such solvent there is substantially no distortion through swelling of the threads, and consequently the spaces between the threads are uniformly left open. The maintenance of these spaces is particularly desirable when rubber is applied to the fabric as it flows therethrough and upon subsequent vulcanization "rubber rivets" are formed. The process has also been found to coat the individual fibers without depositing an excess of lubricant therebetween. Thus the flexibility of

the treated material is not impaired and the formation of the "rubber rivets" mentioned is not interfered with. The advantages mentioned due to the use of an organic solvent are also secured where a naturally coated material is treated with such solvent for forming lubricated joints.

The material resulting from the addition of lubricant has been found to be peculiarly adapted to withstand deteriorating agents which may act upon it during the vulcanizing process. Fabric under ordinary conditions which still retains its natural covering of wax is adapted to withstand the action of vulcanizing agents to some extent, but by the present process this resistance is vastly increased. The resultant resistance to wear through flexing and abrasion of the material is greatly heightened both where lubricant is added and where simple treatment of the fiber with solvent is carried on. A particular advantage of this increased resistance resides in the fact that a less strong cotton fabric may be employed in the manufacture of tire fabrics. At the present time practically all tire fabrics are manufactured from Egyptian or sea island cotton which has a long staple fiber. Short staple cotton such as American upland or peeler cotton is not sufficiently wear-resisting for the manufacture of high-grade tire fabrics. By the present process these short-staple cottons may be employed since their resistance to wear may be increased to equal substantially that of the Egyptian and sea island cotton. Such substitution of the short-staple cotton, of course, effects a relative saving in the cost of the tires.

The process may also be applied to fibers such as hemp, jute, and the like which have no natural waxy coating to impart to them the lubricant with the resulting resistance to abrasion which as heretofore noted is present to some extent in cotton.

As many apparently widely different embodiments of this invention may be made without departing from the spirit thereof, it is to be understood that I do not intend to limit myself to the specific form of the invention as set forth except as indicated in the appended claims.

Having thus described my invention what I claim and desire to protect by Letters Patent is:

1. The process of treating fibrous material which comprises applying thereto a substantially non-drying oil serving as a lubricant dissolved in a volatile solvent, evaporating the solvent and treating the so prepared material with a vulcanizable plastic, the proportion of the oil being relatively small to obviate deleteriously affecting the bond between the fiber and plastic.
2. The process of treating fibrous mate-

- rial which comprises applying thereto a lubricant dissolved in a volatile solvent, evaporating the solvent and treating the so prepared material with a vulcanizable plastic, the proportion of the lubricant being relatively small to obviate deleteriously affecting the bond between the fiber and plastic.
3. The process of treating fibrous material which comprises applying thereto an oil containing wax serving as a lubricant dissolved in a volatile solvent, removing the solvent, and treating the so prepared material with a vulcanizable plastic, the proportion of the oil being relatively small to obviate deleteriously affecting the bond between the fiber and plastic.
4. The process of treating fibrous material which comprises applying thereto a lubricant dissolved in an organic solvent in sufficient quantity to coat the fabric while maintaining the spaces normally present between the fibers substantially open, and treating the so prepared material with a vulcanizable plastic, the proportion of the lubricant being relatively small to obviate deleteriously affecting the bond between the fiber and plastic.
5. The process of treating fibrous material which comprises applying thereto an oil serving as a lubricant dissolved in a solvent, removing the solvent, and treating the so prepared material with a coating of vulcanizable rubber, the proportion of the oil being relatively small to obviate deleteriously affecting the bond between the fiber and rubber.
6. The process of treating fibrous material which comprises applying thereto a quantity of oil and wax sufficient to coat the fibers while maintaining the spaces normally present between the fibers substantially open, and treating the so prepared material with a plastic, the proportion of the oil being relatively small to obviate deleteriously affecting the bond between the fiber and plastic.
7. The process of treating fibrous mate-
- rial which comprises applying thereto a lubricant including castor oil and beeswax and treating the so prepared material with a coating of rubber.
8. The process of treating fibrous material which comprises applying thereto a lubricant including wax dissolved in a solvent, removing the solvent, and treating the so prepared material with a coating of rubber.
9. As an article of manufacture fibrous material having the individual fibers coated with a waxy lubricant in sufficient quantity to cover the fibers while maintaining the spaces normally present between the fibers substantially open, and a layer of rubber intimately associated with the fibrous material, the proportion of the lubricant being relatively small to obviate deleteriously affecting the bond between the fiber and rubber.
10. As an article of manufacture fibrous material evenly coated with an oil in sufficient quantity to cover the fibers while maintaining the spaces normally present between the fibers substantially open, and a layer of rubber intimately associated with the fibrous material, the proportion of the oil being relatively small to obviate deleteriously affecting the bond between the fiber and rubber.
11. As an article of manufacture a layer of fibrous material impregnated by a lubricant residue from a solution containing wax and a layer of rubber intimately associated with the fibers, the proportion of the lubricant being relatively small to obviate deleteriously affecting the bond between the fiber and rubber.
12. As an article of manufacture, fabric, a mixture of oil and wax residue from a solution impregnating said fabric, and a layer of rubber intimately associated with said fabric.

Signed at Newark, county of Essex, and State of New Jersey, this 20th day of June, 1919.

ALFRED E. JURY.